

June 9, 1931.

W. S. BAYLIS

1,808,755

## PROCESS OF TREATING BEESWAX

Filed May 11, 1926



INVENTOR:  
WALTER S. BAYLIS,  
BY *Fred W. Danie*

## UNITED STATES PATENT OFFICE

WALTER S. BAYLIS, OF LOS ANGELES, CALIFORNIA, ASSIGNOR, BY MESNE ASSIGNMENTS, TO FILTROL COMPANY OF CALIFORNIA, A CORPORATION OF CALIFORNIA

## PROCESS OF TREATING BEESWAX

Application filed May 11, 1926. Serial No. 108,269.

My invention relates to bleaching processes and particularly to a process of bleaching and purifying beeswax. Beeswax in its natural condition is of brownish color and contains a certain amount of impurities. In this natural condition it is not of much commercial value, but when this beeswax is bleached to a white color and the impurities are removed it is very useful in many arts.

10 It is an object of this invention to provide a process of bleaching beeswax, which process is very effective in thoroughly bleaching the beeswax to a white color.

Another object of the invention is to provide a process of bleaching beeswax which is economical and expeditious.

I have discovered that a better product is obtained if the process is carried on under a vacuum.

20 It is accordingly one of the objects of this invention to provide a process of bleaching beeswax which is carried on under a vacuum.

Other objects and advantages of the invention will be made manifest hereinafter.

25 Referring to the drawing in which I illustrate an apparatus for conducting my invention,

Numeral 1 denotes a heater, 2 denotes a washer, 3 denotes a primary mixer, 4 denotes 30 a conveying pump, 5 denotes a primary bleaching tank, 6 denotes a primary pressure pump, 7 denotes a primary filter press, 8 denotes a secondary mixer, 9 denotes a secondary bleaching tank, 10 denotes a secondary 35 pressure pump, 11 denotes a secondary filter press, 12 denotes a storage tank, 13 denotes a liquid trap, 14 denotes a condenser, and 15 denotes a vacuum pump.

The heater 1 has a shell 20 which is fitted 40 with a steam coil 21. The shell 20 has a conical bottom 24 which is drained by a pipe 25 having a valve 26.

The washer 2 consists of a shell 30 which 45 provides a washing chamber 31 and which is surrounded by a heating jacket 32. The washing chamber 31 is closed by a tight cover 33. Adapted to rotate in the chamber 31 are agitating paddles 35. A tightly covered opening 36 is provided in the cover 33 for the introduction of beeswax into the

chamber 31 for treatment. The pipe 25 passes through the cover 33 and connects with the chamber 31. The shell 30 has a conical floor 38 which is drained by a pipe 39 which terminates its lower end in a T fitting having valves 40 and 41 at its opposite ends. A pipe 42 leading from the valve 41 empties into the open upper end of a shell 45 which forms a mixing chamber 46 in the primary mixer 3. Agitating paddles 47 are provided in the chamber 46 and are adapted to be rotated therein. A valved hopper 48 opens downwardly over the upper open end of the shell 45. The shell 45 has a conical bottom 50 having a drain pipe 51 which is provided with a valve 52 and connects with the intake end of the conveying pump 4.

The primary bleaching tank 5 has a shell 55 which forms a bleaching chamber 56 and has 70 a steam jacket 57 for heating the contents of this chamber. Agitating paddles 58 are located in the bleaching chamber 56 and are adapted to be rotated therein. The top of the shell 55 is provided with a tight cover 60 which has a tightly covered opening 61 provided therein. A pipe 62 connects the exhaust end of the conveying pump 4 to an opening in the cover 60 so as to communicate with the chamber 56. The shell 55 has a 75 conical bottom 65 which has a drain pipe 66 which has a valve 67 and which connects to the intake end of the primary pressure pump 6. The exhaust end of the pump 6 is connected by a pipe 70 to a shell 72 of the 80 primary filter press 7. The shell 72 provides a filter chamber 73 in which are disposed filter plates 74 which are connected through the shell 72 by pipes 75 to a header 76. The header 76 has a valve 78 which connects with 85 a pipe 79 which empties into the open upper end of the secondary mixer 8. The secondary mixer 8 has a shell 81 which provides a mixing chamber 82 in which agitating paddles 83 are disposed, these being adapted to 90 be rotated. A valved hopper 85 empties into the upper end of the shell 81. The shell 81 has a conical floor 86 which is provided with a drain pipe 87 which has a valve 89.

The secondary bleaching tank 9 has a shell 10

90 which provides a secondary bleaching chamber 92 in which agitating paddles 93 are disposed, the paddles 93 being adapted to be rotated. A steam jacket 94 is disposed about the shell 90 for heating the contents of the chamber 92. A tight cover 96 closes the upper end of the shell 90. The drain pipe 87 is fitted tightly into an opening in the cover 96 so as to connect with the chamber 92. A tightly covered opening 98 is provided in the cover 96 for a purpose which will be described later. The shell 90 has a conical bottom 100 which is provided with a drain pipe 101 having a valve 102 and which connects to the intake end of the secondary pressure pump 10. A pipe 105 connects the exhaust end of the secondary pressure pipe 10 to a shell 106 of the secondary filter press 11. The secondary filter press 11 is identical with the primary filter press 7 and filtrate is conducted therefrom through a header 107 which has a valve 108. A pipe 109 leads from the valve 108 and empties into the storage tank 12. The storage tank 12 is provided with a heating coil 112 for a purpose which will be described later. An outlet pipe 113 which has a valve 114 is provided in the lower end of the storage tank 12.

The condenser 14 is diagrammatically shown as a condenser of standard construction having a tight shell 120 in which upper and lower secondary heads connected by tubes as indicated by dotted lines are provided. The shell 120 has a conical bottom 122 which is provided with a drain pipe 123 having a valve 124. Connecting with the condenser shell 120 at a point just below the lower of these secondary heads is a vacuum pipe 125 of the vacuum pump 15. A pipe 126 connects the upper end of the condenser 14 with the water trap 13. Leading from the water trap 13 is a vacuum line 127 which has a branch line 128 provided with a valve 129 and which passes through an opening in the tank cover 60 to connect with the primary bleaching chamber 56 of the primary bleacher 5. The vacuum line 127 also has a branch line 130 which has a valve 131 and which connects with the secondary bleacher 9 to communicate with the secondary bleaching chamber 92. The vacuum line 127 has another branch line 135 which has a valve 136 and which connects with the upper end of the storage tank 12. When the vacuum pump 15 is set in operation, a vacuum is imposed upon the condenser 14 and, through the pipe 126, the water trap 13, the vacuum line 127 and its branches 128, 130 and 135, upon the primary bleaching chamber 56, the secondary bleaching chamber 92, and the interior of the storage tank 12.

The process of the invention is carried on as follows:

At the time the process is started, all of the valves shown in the above described appara-

tus are closed. The beeswax in its natural form is introduced into the washer 2 through the opening 36. The vacuum pump 15 may at this time be set into operation so that the interiors of the different pieces of apparatus will be subjected to a vacuum. The heating jacket 32 is supplied with a suitable heating medium, such as steam, for the purpose of raising the temperature of the washing chamber 31 so that the beeswax will be melted. When the beeswax has been melted, a treating fluid is introduced into the mixing chamber 31 through the pipe 25. This treating fluid preferably consists of a solution of sulphuric acid and water, which ingredients are supplied to the heater 1 through the pipes 22 and 23 respectively. From experience I have found that a very satisfactory treating fluid is made from one part of 66 per cent sulphuric acid and four parts of water. After the proper mixture of acid and water has been made in the heater 1, steam is passed through the coils 21 so as to heat the treating fluid to about the temperature of the beeswax when the wax has been liquefied in the washing chamber 31. The valve 26 is then opened. The agitating paddles 35 are at this time set into operation and the beeswax is slowly stirred during the time that the treating fluid flows through the pipe 25 into the mixing chamber 31. Sufficient treating fluid should be added to the beeswax to provide approximately 2 per cent by weight of 66 per cent sulphuric acid as compared to the weight of beeswax being treated.

The temperature of this mixture is then gradually raised to about 214° F., at which temperature it is held for about five minutes. During this period of high temperature the mixture of treating fluid and beeswax is slowly agitated, and the treating fluid takes a part of the color constituents and impurities from the beeswax. The agitation is then stopped and the mixture is allowed to settle. The treating fluid is heavier than the wax and will occupy the extreme lower part of the mixing chamber 31 when settling takes place. Due to the fact that the treating fluid has absorbed considerable of the impurities of the wax, the stratum of beeswax above the stratum of treating fluid will be much lighter in color than the wax when first placed in the chamber 31. The valve 40 is now opened and the lower stratum 140 in the chamber 31, composed of treating fluid and sludge, is drawn off.

When the upper stratum 141 in the chamber 31 which is composed of melted beeswax begins to flow from the valve 40, this valve is closed and the valve 41 is opened. The melted beeswax then flows from the chamber 31 through the pipe 42 into the primary mixer 3. The paddles 47 are set in operation and as the mixing chamber 46 fills with melted beeswax, a decolorizing mineral is fed

into the beeswax from the valved hopper 48. This decolorizing mineral is preferably a chemically prepared absorptive clay such as is at present used in the refining of mineral and vegetable oils. Although various quantities may be effectively used, I prefer to add a percentage of 20 per cent of decolorizing mineral by weight. As soon as the decolorizing mineral is thoroughly mixed with the melted beeswax, the valve 52 is opened and the conveying pump 4 set in motion to transfer the mixture of beeswax and mineral to the primary bleaching chamber 56. The mixer 3 may be of sufficient size to mix a whole batch at once or else the transfer of beeswax and mineral to the primary bleaching tank 5 may be commenced before all of the wax has flowed from the washer 2. It is not necessary that a complete mixing of wax and mineral take place in the mixer 3, this element of the apparatus merely being used to prevent excessive foaming of the mixture in the primary bleaching tank 5. Before the mixture is delivered to the chamber 56, the valve 129 is opened and a vacuum is thus placed in the chamber 56. I have found that no foam will form in the chamber if the mixture is introduced when there is a vacuum.

In the chamber 56 the mixture of decolorizing mineral and beeswax is then thoroughly agitated by setting the agitating paddles 58 into operation. During this agitation a heating medium, such as steam, is supplied to the heating jacket 57, and the temperature of the mixing chamber 56 is raised to about 300° F. During this rise in temperature and this agitation, the decolorizing mineral is brought into intimate contact with the beeswax and practically all of the impurities and color constituents are absorbed or adsorbed therefrom. After this agitation has taken place for a sufficient period for the reaction to be completed, the valve 67 in the pipe 66 is opened, and the primary pressure pump 6 is set into operation in order to force the mixture of beeswax and decolorizing mineral into the primary filter press 7. The mixture from the bleaching chamber 56 is forced into the filter chamber 73 provided by the shell 53. The beeswax which, of course, is in the form of a liquid will pass through the filter plates 74, the pipes 75 and into the header 76. The decolorizing material, however, is too coarse to pass through the filter plates and will collect thereon in the form of cakes as indicated at 150. These cakes 150 contain all the impurities and color constituents which have been removed from the beeswax.

The valve 78 is now opened and the filtered beeswax is carried by the pipe 79 to the mixing chamber 82 of the secondary mixer 8. Here fresh decolorizing mineral poured from the valved hopper 85 is mixed with the melted beeswax in the same manner as a similar mixture was made in the primary mixer 3. As

this mixing proceeds, the valve 89 is opened to allow the mixture to pass by gravity into the mixing chamber 92 of the secondary bleaching tank 9. The valve 131 has been previously opened so there is a vacuum in the chamber 92 when the mixture enters; therefore, there will be no foam. The paddles 93 are set into operation in order to thoroughly mix the beeswax and the decolorizing mineral, and the heating jacket 94 is supplied with a heating medium in order to raise the temperature of the mixing chamber 92 to a temperature of about 300° F. The action which takes place in the mixing chamber 92 is substantially the same as the action which has taken place in the mixing chamber 56.

The beeswax when it has reached the secondary bleaching tank is very nearly bleached and contains but a very small percentage of impurities. The treatment in the secondary bleaching tank will thoroughly remove any of the impurities or color elements which remain, these being absorbed or adsorbed by the fresh decolorizing mineral. After a certain period of time has elapsed, the valve 102 is opened and the pump 10 is put into operation, thus pumping the mixture from the mixing chamber 92 to the secondary filter press 11 where the beeswax is filtered from the decolorizing mineral. The action in the secondary filter press is identical with the action which takes place within the primary filter press 7. The valve 108 is opened and the beeswax is passed through the pipe 109 to the storage tank 12, ready to be cooled. The beeswax is kept at a temperature sufficient to keep it from solidifying in the tank 12 by means of the steam coil 112, and it may be withdrawn from the tank through the pipe 113 by opening the valve 114. When the beeswax reaches the storage tank 12 it is thoroughly bleached and all of the impurities and color constituents have been removed therefrom. The beeswax at this time is practically pure white.

In conducting the process I find it economical to use a "spent" decolorizing mineral in the primary bleaching tank 5, that is to say, the decolorizing mineral which has been collected in the secondary filter press 11 is not discarded but is used in the primary bleaching tank 5. This is economical due to the fact that the decolorizing material obtained from the secondary filter press 11 still has considerable power of adsorption. I find that the product is better when the process is conducted under vacuum. This is probably due to the fact that any breaking down of molecules is prevented by reason of an absence of air in the different apparatus.

It should be understood that the drawing shows the apparatus very diagrammatically, and may have additions as desired. For instance, it may be advantageous to have heating means for the filter presses and mixers

3 and 8 to eliminate a possibility of solidification of the beeswax. The apparatus shown, however, is essentially adequate for carrying out the novel process of my invention.

5 Some light waxes may be treated sufficiently by an acid wash and one "contact" with the bleaching agent, as in the primary bleaching tank 5, so that they may be run directly to storage upon leaving the primary filter press 7. The double bleaching contact is shown for the purpose of illustrating the process followed in treating the darkest form of beeswax it will be necessary to handle.

10 It should be understood also, that the primary and secondary mixers 3 and 8 are a helpful but not an essential step in the process of this invention. In case these mixers were dispensed with, the bleaching agent would be placed in the bleaching tanks 5 and 9 through the openings 61 and 98, and the wax would be introduced into the bleaching tanks gradually to keep down the foaming which has a tendency to accompany the mixing of the beeswax with the bleaching

15 agent.

20 I claim as my invention:

25 1. A process of bleaching beeswax comprising: melting the beeswax; agitating said beeswax with dilute sulphuric acid; settling out said dilute acid; treating under vacuum said liquefied beeswax with a decolorizing agent comprising an acid-activated colloidal clay at a temperature approximating 300 degrees F.; and separating said decolorizing agent from said beeswax at a temperature approximating 300 degrees F.

30 2. A process of bleaching beeswax comprising: heating the beeswax sufficiently to cause it to melt; heating a dilute sulphuric acid solution to approximately the same temperature as said beeswax; mixing said beeswax and said treating fluid; raising the temperature of the beeswax and treating fluid to about 214° F.; settling said treating fluid from said beeswax; removing said beeswax; mixing said beeswax with a decolorizing agent comprising an acid-activated colloidal clay at a temperature approximating 300 degrees F.; and filtering said decolorizing agent from said beeswax, said decolorizing steps

35 being performed under vacuum.

40 45 50 In testimony whereof, I have hereunto set my hand at Los Angeles, California, this 6th day of May, 1926.

WALTER S. BAYLIS.